

## UNITED STATES PATENT OFFICE

MAX SCHLÖTTER, OF BERLIN, GERMANY, ASSIGNOR TO ASOCIACION DE PRODUCTORES  
DE YODO DE CHILE, OF VALPARAISO, CHILE

## ELECTROLYTIC SEPARATION OF COPPER

No Drawing. Application filed September 28, 1929, Serial No. 396,003, and in Germany October 29, 1928.

Since double the electrochemical equivalent of copper can be separated from solutions of cuprous salts compared with those of cupric salts, attempts have been made to obtain usable copper deposits for example from cuprous chloride ( $CuCl$ ). It has been found however that cuprous chloride solution easily oxidizes in the presence of air and cupric chloride ( $CuCl_2$ ) is formed through which the quality of the copper deposit as is well known is reduced, while with increasing content of cupric chloride the yield decreases and finally constancy of yield can no longer be depended on, which is a considerable disadvantage in practical operation.

Accordingly all kinds of methods have been proposed for avoiding the oxidisation of the electrolyte; for example the surface of the liquid has been protected from the air by an air tight layer of paraffin or the like. All these prior proposals for keeping away the oxygen of the air make the operations with the electrolyte more difficult and in many cases hinder the production of a uniform deposit.

The use of cuprous chloride solution therefore does not enable the desired technical result to be obtained.

It has now been found that solutions of cuprous iodide ( $CuI$ ) are particularly suitable for the separation of copper. Any cupric iodide ( $CuI_2$ ) which may be formed splits up into cuprous iodide and iodine which additively combines with the solvent. The electrolysis can be carried out without exclusion of air, so that all the above mentioned measures which render the operations difficult are unnecessary.

Since cuprous iodide is not easily soluble in water, it has been found advantageous to dissolve the cuprous iodide with the addition of such other salts as increase its solubility. It has been found that cuprous iodide is so soluble when accompanied in particular by the halogenides of alkali, and alkaline earth, metals, chiefly the iodides, and also by sulphites, thiosulphates, cyanides and the like, that current densities of 400 amps./sq. meter and upwards can be

used without the properties of the cathode copper being harmfully affected. In spite of the high content of alkali, or alkaline earth metal there is no liberation of hydrogen at the cathode. Solution of the anode, in spite of the low solubility of cuprous iodide in water, takes place steadily and quantitatively, and the cuprous content of the electrolyte remains constant. The process takes place quantitatively at the anode as well as at the cathode.

Even with rapid circulation of the electrolyte, no harmful oxidisation thereof takes place.

The above described process of copper separation can be used with equally satisfactory results in the plating of metal objects with copper, in the making of electrolytes and in the refining of black copper.

By way of example a bath of the following composition can be used in carrying out the process: 1,000 c. c. water, 600 gms.  $KI$ , 60 gms.  $CuI$ .

With this bath a pressure of about 0.3 volts and a current density of about 400 amps./sq. meter are used.

It has further been found that colloids or capillary active substances can be added to the cuprous iodide solution in order to obtain bright and smooth coatings, without the metal becoming brittle, as occurs for example with the addition of these substances to copper sulphate solution. Among colloids, glue, gelatine and the like and among capillary active substances, phenols, tannin and the like, have been found particularly suitable, used in quantities of 5-10 gms. per liter of the bath.

What I claim is:

1. A method of separating copper which consists in electrolyzing an aqueous solution containing cuprous iodide.

2. A method of separating copper which consists in electrolyzing an aqueous solution containing cuprous iodide without excluding air from contact with the solution.

3. A method of depositing copper which consists in electrolyzing an aqueous solution containing cuprous iodide in contact with the atmosphere.

4. A method of separating copper which consists in electrolyzing an aqueous solution containing cuprous iodide and a salt of an alkali or alkaline earth metal.
5. A method of separating copper which consists in electrolyzing an aqueous solution containing cuprous iodide and a halogenide of an alkali or alkaline earth metal.
6. A method of separating copper which consists in electrolyzing an aqueous solution containing cuprous iodide and an iodide of an alkali or alkaline earth metal.
7. A method of separating copper which consists in electrolyzing an aqueous solution containing cuprous iodide and potassium iodide.
8. A method of separating copper which consists in electrolyzing a solution containing cuprous iodide and potassium iodide without excluding air.
9. A method of separating copper which consists in electrolyzing a solution containing cuprous iodide and potassium iodide with a copper anode, without excluding air.
10. An electrolyte for the electrolytic separation of copper comprising an aqueous solution containing cuprous iodide.
11. An electrolyte for the electrolytic separation of copper comprising an aqueous solution containing cuprous iodide and an alkaline iodide.

In testimony whereof I have signed my name to this specification.

MAX SCHLOTTER.

35

40

45

50

55

60